

## UNITED STATES PATENT OFFICE

2,441,496

## LUBRICATING OILS

Bert H. Lincoln, Ponca City, Okla., Gordon D. Byrkit, Niagara Falls, N. Y., and Waldo L. Steiner, Ponca City, Okla., assignors to Continental Oil Company, Ponca City, Okla., a corporation of Delaware

No Drawing. Application November 9, 1942,  
Serial No. 465,094

20 Claims. (Cl. 252—46.6)

1

This application is a continuation-in-part of our copending application Serial No. 283,570, filed July 10, 1939, which has since issued into Patent No. 2,348,030, dated May 2, 1944.

Our invention relates to lubricating oils and more particularly to an improved lubricating oil of general utility which has a high film strength, is noncorrosive to the crankcase bearing materials and does not readily oxidize or form sludges and lacquers.

In the development of new automotive and other type engines, increased power, higher oil temperature, increased bearing pressures per unit area, and other innovations have led to the installation of bearings made of new bearing materials, alloys and mixtures, which unfortunately are more readily attacked by oxidation products formed in the lubricant than was the old Babbitt bearing metal. Some of these newer bearing materials are cadmium-silver, copper-lead, and alloys of lead with other metals. These metals are corroded readily by oils which have been used for a relatively short time in the engine. Oils which have been solvent refined or otherwise refined to produce oils with high viscosity indexes (for example, 93 V. I. or higher) are characterized by a deficiency of natural oxidation inhibitors and consequently are especially subject to oxidation which forms corrosive organic acids and pro-oxidation catalysts which promote the further oxidation and deterioration of the oil. These oils also have an objectionable characteristic in that they tend to deposit lacquerous formations upon the various engine parts, particularly the piston ring, ring grooves, and skirt. Ring sticking, poor heat radiation, and reduced lubrication cause accelerated wear and eventual engine failure. One method of overcoming the injurious bearing composition loss caused by corrosion would be to use more resistant bearing compositions and another would be to use an oil which does not develop these corrosive materials during use. Still another method would be to use a lubricant containing a material which would react with and render inert the oxidation products which promote oil deterioration and oxidation as rapidly as they are formed. Lacquer formation with the resultant ring-sticking, failure of proper radiation of heat with the resultant piston and cylinder wall warping, cylinder wall scuffing, piston slap, etc., may often be prevented or reduced by adding a compound having that characteristic known as detergency. Such detergency compounds are metal organic compounds such as metal soaps, a metallo-organic compound, or a phosphorus compound to the oil.

2

Various addends have also been proposed for addition to lubricants for the purpose of inhibiting the formation of oxidation products during use. These may be called antioxidants, since they increase the induction period or that period of time before which oxidation begins and decrease the rate of oxidation after it has started.

Other organic compounds have been added to a lubricating oil to increase the film strength of the oil, thus allowing smaller bearing areas to support the same or heavier loads without the danger of the oil being squeezed from between the rubbing surfaces. These compounds are especially necessary in lubricating the modern hypoid gears and have proved to be very beneficial when used in the crankcases of high-powered internal combustion engines.

Our invention is not concerned with the first mentioned methods of reducing bearing metal loss, that is, use of more resistant bearing metals and the use of noncorrosive and nonoxidizing oil, but is concerned with the other methods of improving a lubricant.

The present invention proposes the addition of two addends to a lubricant which has been found to give the lubricant an unexpectedly superior activity in respect to film strength, corrosion inhibition, and lacquer prevention over what would be expected from simply the postulated effect of the combination upon a lubricant from a knowledge of the effect of each of the addends used separately upon the oil.

Certain compounds when added to oils are physically or chemically held by, or otherwise combined with metals, forming tenacious films on the surface of the metals which enable them to withstand higher pressures without the welding of one metal surface to the other. The various chlorine and sulfur compounds are the most noteworthy of this type of compound and because of their activity are known as "extreme pressure" and "mild extreme pressure" addition agents.

Furthermore X-ray diffraction methods have shown that compounds having highly polar molecules, that is, molecules of unsymmetrical character containing an atom or group of atoms exhibiting a secondary or residual valence, tend to produce regimentation of the polarized molecules in a hydrocarbon oil upon the surface of metals immersed in the oil. The coefficient of friction of the oil is reduced by the orientation of the molecules. An oil exhibiting a low coefficient of friction for the viscosity thereof is known as an oil having a high oiliness factor.

One object of our invention is to provide a substantially noncorrosive lubricant for use with the

new, easily corroded bearing compositions. It is to be noted, however, that the improved lubricants here described are advantageously employed with all types of bearings, since they are less corrosive during use with any of the metals commonly encountered in practice and have properties apart from noncorrosiveness which designate them of great utility for many lubrication purposes.

Another object of the invention is to provide a lubricant inhibited against oxidation during use.

Another object of our invention is to provide a lubricant characterized by high film strength as compared with plain or refined mineral lubricating oils.

A further object of the invention is to provide a lubricant containing an addend capable of reacting with or otherwise rendering inert such products of oxidation and corrosion as may be formed during extended use and such catalytically active metallic elements or compounds as may via blow-by, etc., become a contaminant of the lubricant.

Another object of the invention is to provide a lubricant which will not form undesirable lacquer and varnish coatings upon various parts of the piston and the parts of the engine cooperating therewith as readily as such deposits are formed by the refined mineral lubricating oils.

Another object of the invention is to provide a lubricant characterized by its ability to maintain sludge, polymerization products, and insoluble contaminants in a state of colloidal suspension as distinguished from sludge or insoluble contaminants precipitated or deposited on the various parts of the engine.

Another object of our invention is to provide a lubricant of high oiliness characteristics.

Other objects of our invention will be apparent in the following description.

Our invention comprises an improved lubricating composition of especial utility for the lubrication of the bearing and frictioning surfaces of modern internal combustion engines, although, as noted above, it is not limited to such specific use. The lubricating composition comprises an oil of lubricating viscosity and two additives of unrelated properties which coact with the oil and each other to give a lubricating composition of superlative characteristics with respect to the most important properties of a lubricant to be used in the crankcase of an internal combustion engine.

One of the compounds of the invention is a sulfurized relatively high molecular weight olefin, the olefin being selected from the group of unsaturated organic compounds consisting of naturally occurring unsaturated mineral oils, vegetable oils, and animal oils, and the esters of their fatty acids, and manufactured oils, such as dehydrogenated oils, halogenated and dehydrohalogenated oils, cracked hydrocarbons, and similar olefins. More particularly the compound may be sulfurized corn oil, sulfurized cottonseed oil, sulfurized rapeseed oil, sulfurized castor oil, sulfurized lard oil, sulfurized sperm oil, and the sulfurized esters of their fatty acids, sulfurized cracked wax, sulfurized cracked gasoline, sulfurized olefin obtained from narrow-cut liquid petroleum fractions, such as kerosene, gas oil, neutral oil, etc., or sulfurized olefin obtained by halogenating and dehydrohalogenating a petroleum wax.

The preferred compound is the sulfurized olefin

obtained by halogenating a petroleum wax whose monochloro derivative melts at a lower temperature than does the hydrocarbon itself, separating respectively the monochloro, dichloro, and more highly chlorinated derivatives from the unchlorinated wax and from the less highly chlorinated and more highly chlorinated hydrocarbons, dehydrohalogenating the relatively pure monochloro wax derivative or the dichloro wax derivative to obtain a relatively pure, homogeneous olefin. The sulfurization of the olefin is by means of a sulfurizing agent which may be elemental sulfur or a sulfur compound such as sulfur chloride, etc. This particular compound and the method of making the same are fully described in the United States Patent No. 2,218,032, issued October 5, 1940, upon the application of Bert H. Lincoln, Waldo L. Steiner, and Gordon D. Bykit, Serial No. 205,531, filed May 2, 1938.

The other compound to be added to the lubricant is selected from the broad group of organic phosphorus compounds and may, in general, be any organic phosphorus compound having a sufficiently high boiling point to allow its incorporation and maintenance in a lubricant to be subjected to the heat conditions present in the crankcase of an internal combustion engine. It has been found that all phosphorus-containing organic compounds of sufficient boiling point under atmospheric pressure to insure their continued presence in a lubricant enhance the activity of the sulfurized olefin in the lubricant and in other respects produce a lubricant of improved quality. The phosphorus compounds may be broadly any organic phosphorus compound, and the phosphorus may be in its trivalent or pentavalent form, the phosphorus compound may consist only of phosphorus, hydrogen, and carbon or it may contain in addition thereto an element or elements from the group consisting of oxygen, sulfur, tellurium, selenium, nitrogen, chlorine, and metals such as calcium, sodium, barium, tin, lead, zinc, aluminum, antimony, arsenic, lithium, etc. The phosphorus compound may be an ester of an acid of phosphorus or a compound having the phosphorus directly attached to one or more carbon atoms. The organic radical or radicals of the compound may be aliphatic, aromatic, heterocyclic, saturated, or unsaturated. In general, we have found that any organic compound characterized by the presence therein of phosphorus may be advantageously used in the practice of this invention. Particular classes and compounds within the broad class of organic phosphorus compounds are more effective addition agents for our purposes than are other organic phosphorus compounds; however all of the compounds are of some utility in the practice of our invention.

By the combination of the two additives, the oil fortified therewith is improved more than would be expected from the study of the effect of the oil plus sulfurized olefin and an oil plus an organic phosphorus compound. The unexpected improvement will become apparent during the course of the following description.

As little as 0.05 per cent of the combination of the sulfur compounds and organic phosphorus compounds may be added to a lubricant with beneficial results therefrom in respect to resistance to oxidation, reduction in corrosiveness, and capability to maintain insoluble material in a state of colloidal suspension and in other important respects. As much as 20 per cent of the combination of sulfurized olefins and organic

phosphorus compounds may be added to a lubricant to obtain a lubricant exhibiting markedly increased film strength, oiliness properties, prevention of sludges and lacquer-like varnish deposits, and resistance to oxidation and deterioration. It is seldom, however, that more than 2 per cent need be used for a crankcase lubricant. A lubricant containing from 2 to 20 per cent makes an admirable cutting oil or an extreme pressure lubricant.

#### THE SULFUR COMPOUND

As above stated, relatively high molecular weight sulfur compounds suitable for the practice of this invention may be obtained by sulfurizing naturally occurring hydrocarbon olefins which may be an animal oil, such as sperm oil, lard oil; a semi-drying or non-drying vegetable oil, such as corn oil, castor oil, cottonseed oil, rapeseed oil, palm oil, soya bean oil, etc., or the esters of their unsaturated fatty acids or by sulfurizing olefins produced by treating naturally occurring waxes, relatively pure high molecular weight paraffinic substances, narrow-cut liquid petroleum fractions, and petroleum wax, the treating being dehydrogenation, cracking, or halogenation and dehydrohalogenation. All of these sulfurized olefins have been added to lubricating compositions to improve the oil's resistance to oxidation or to reduce the corrosiveness of the oil which is subjected to oxidizing conditions. The most efficacious compound so far discovered for most purposes is the relatively pure sulfurized olefin obtained from petroleum wax by halogenation, separation, and dehydrohalogenation. The preparation of this compound is described in the United States Patent No. 2,218,132, mentioned above. The narrow-cut liquid petroleum fraction such as Stoddard's solvent, a narrow cut of kerosene, a narrow cut of distillate, a narrow cut gas oil, a narrow cut of gasoline, a narrow cut of a highly solvent-treated low (neutral) or high (bright stock) viscosity oil, etc., may be treated in the same manner, that is, by halogenation, separation, and dehydrohalogenation, to produce an olefin suitable for sulfurization and use in our invention.

In order to fully describe the sulfur compound, the method of preparation of the preferred sulfurized petroleum wax, having about 18 to 24 carbon atoms, is herebelow set forth:

First, in order to more fully understand the invention and improvement thereof over the prior art, it is desirable to consider the prior art relating to sulfurized olefins obtained from petroleum wax. References are therein made to monochloro paraffin, dichloro paraffin, and the like, usually considering the product of direct chlorination to be the compound represented by the total chlorine content and therefore the desired compounds. We have found that these materials are very crude mixtures of the chlorinated hydrocarbons and contain unchlorinated hydrocarbons and the mono-, di-, and polychloro derivatives and cannot be considered the desired compounds. For example, a so-called "trichloro paraffin wax" containing 24 per cent chlorine, which corresponds very closely to percentages of chlorine in the trichloro compound, was separated by means of crystallization from acetone, the first (least soluble) portion consisting of a mixture of monochloro wax and unchlorinated wax. The percentage of unchlorinated wax in the original mixture was found to be 7.2 per cent; thus even a "trichloro paraffin" as so called in the prior

art because of the total chlorine content was in fact a crude mixture containing as much as 7.2 per cent of unchlorinated wax, and more highly chlorinated waxes. Its use would not give the homogeneous sulfurized products that are obtained from a relatively pure homogeneously halogenated paraffin wax.

As stated above, the relatively pure mono- or diolefin free from unchlorinated hydrocarbons and free from more highly chlorinated hydrocarbons may be prepared by halogenation, separation, and dehydrohalogenation.

To produce a maximum amount of monochloro wax, about 10 per cent of chlorine is added to the petroleum wax having from 18 to 24 carbon atoms and a melting point of approximately 120° F. The other halogens may be used in place of the chlorine, but we prefer chlorine because of its availability and cheapness. As stated above, the chlorinated mass will contain unchlorinated wax. The chlorination of wax varies its melting point stepwise inversely as the degree of chlorination. The monochloro wax melts lower than the unchlorinated wax. The dichlorinated wax melts lower than the monochlorinated wax. By making use of this difference in melting points or differences in solubility, it is possible to separate readily the unchlorinated wax from the crude chlorination mixture, using sweating or selective solvent treating at various temperatures. Then the monochloro wax may be separated from the mixture of monochloro and more highly chlorinated wax in the same manner. We thus obtain a relatively pure monochloro wax of from 18 to 24 carbon atoms. If it is desired to produce a maximum amount of a diolefin of from 18 to 24 carbon atoms, the process is carried out in the same manner except that 17 per cent chlorine is originally introduced into the wax, and the dichloro wax is separated from the unchlorinated, monochlorinated, and the more highly chlorinated wax.

A solution of the crude-chlorination mixture of chlorinated paraffin wax may be formed with acetone. At about 70° F. the chlorinated waxes will be in solution while the unchlorinated wax will not be dissolved and may be separated out by settling, centrifuging, or filtering. The solution may be chilled to precipitate the monochloro wax. Thus the monochloro wax may be separated from the polychloro wax, employing the same methods outlined for separating the unchlorinated wax from the chlorinated wax mixture.

The monochloro wax thus obtained is substantially a pure monochloro compound, being free from unchlorinated and more highly chlorinated waxes although, of course, the homologues of from 18 to 24 carbon atoms are present and may be converted to the corresponding mono-olefin by removing the chlorine, along with an adjacent hydrogen, as hydrogen chloride, thus producing a mono-olefin. To effect dehydrohalogenation and thus produce the olefin, the monochloro wax may be heated for a period of a minute or less to five hours with  $\frac{1}{10}$  of its weight, more or less of lime, at a temperature of from 200° F. to 500° F. A much lower percentage of lime or other basic material may be employed, although in many cases the higher percentages have been found to give a better colored olefin composition. The olefin may be formed by heating with no basic or other material; however this is not recommended because of the darkened color of the product. This step is defined herein and in the claims as dehydrohalogenation, because the chlo-

rine is removed, together with an atom of hydrogen from a carbon atom adjacent to the carbon atom to which the chlorine was attached, in the form of hydrochloric acid.

As mentioned before, it is possible to employ a relatively pure diolefin obtained from petroleum wax or a narrow-cut petroleum fraction in place of the mono-olefin. Instead of chlorinating to the theoretical chlorine content of a mono-olefin, the chlorination is carried on to the degree at 10 which the wax or narrow-cut petroleum fraction is theoretically a dichloro wax; the dichloro wax or fraction is separated from the unchlorinated wax or fraction and more and less highly chlorinated wax or fraction and dehydrohalogenated.

Having obtained a relatively pure, high molecular weight olefin, the sulfur-bearing addition agent is formed by sulfurizing the olefin or diolefin. The sulfurization may be by means of elemental sulfur or a sulfur compound such as a sulfur chloride, a phosphorus sulfide, or the like. In general, the sulfurized olefins prepared by reacting the olefins with a sulfur compound are more stable than the sulfurized olefins obtained by sulfurizing an olefin with elementary sulfur; however by controlling the temperature and time of reaction and diluent, it is possible to obtain stably bound sulfurized olefins by reacting the olefins with elemental sulfur.

It is to be understood that we do not intend to be limited to the particular sulfurized compound obtained from petroleum wax simply because it is a preferred example of our sulfur compounds. The other petroleum fractions and the animal and vegetable oils and esters of their fatty acids mentioned above are admirably suited for treatment in accordance with the above teaching to give sulfur-bearing compounds which are very effective materials when used in the practice of this invention.

#### THE PHOSPHORUS COMPOUNDS

We have found that in general any organic phosphorus compound may be used in the practice of this invention, although certain organic phosphorus compounds are more effective than other organic compounds. Very small proportions of one or more organic phosphorus compounds may be added to the lubricant containing the sulfurized olefin. In general, it may be said the organic phosphorus compound should be present in an amount ranging from 0.001 per cent to 5 per cent, depending upon the particular phosphorus compound and the oil to which it is added. Higher percentages than this, however, may be desirable in particular cases. The organic phosphorus compound, if it is to be added to a lubricant to be employed in the crankcase of an internal combustion engine, must be sufficiently stable to resist decomposition under conditions present in such a place and it must have a sufficiently high boiling point to prevent its volatilizing and being thus removed from the lubricating composition. Those phosphorus compounds having a vapor pressure of less than atmospheric at 170° F. are satisfactory for all ordinary purposes; and, for some purposes, those having a vapor pressure greater than atmospheric at even lower temperatures are operable.

As stated above, the organic phosphorus compounds may be any organic compound containing phosphorus in its trivalent or pentavalent form. The compound may consist entirely of phosphorus, hydrogen, and carbon, or it may (preferably) contain, in addition to carbon phos-

phorus, and hydrogen, elements such as oxygen, sulfur, tellurium, selenium, nitrogen, chlorine, and metals such as calcium, sodium, barium, tin, lead, zinc, aluminum, antimony, arsenic, lithium, etc. The compound may be a straight ester or mixed ester of an acid of phosphorus and an organic compound which may be aliphatic, carbocyclic, or heterocyclic and which may be saturated or unsaturated. The phosphorus may be joined directly to carbon atoms of the organic radicals or it may be indirectly joined thereto through oxygen, sulfur, and other atoms. The organic phosphorus compound may be the product of the reaction of an organic compound such as a hydrocarbon, or a derivative thereof such as an alcohol, ketone, ester, and ether, in which the compound may be aliphatic or carbocyclic, and an inorganic phosphorus compound such as phosphorus trioxide, phosphorus pentoxide, phosphorus trisulfide, phosphorus pentasulfide, and yellow phosphorus. Compounds containing chlorine are especially effective. In general, we have determined that any organic compound characterized by the presence therein of one or more atoms of phosphorus may be utilized in the practice of this invention; and our invention, therefore, contemplates and environs the use of any such compound.

The following list of organic phosphorus compounds sets forth but a partial list of compounds which may be added to a lubricant in conjunction with a sulfurized olefin to improve the lubricant in respect to very important characteristics normally inadequate in the highly refined and moderately highly refined lubricating oil. This list of compounds is not to be considered a limitation of our invention but is only to be considered as a list of preferred examples of phosphorus compounds and further as representatives of the broad class of organic phosphorus compounds which, as we have indicated above, are effective lubricant addition agents when used for that purpose in conjunction with sulfurized olefins.

#### ORGANIC PHOSPHORUS COMPOUNDS

##### I. Aliphatic

|    |                                              |
|----|----------------------------------------------|
| 50 | Butyl phosphite                              |
|    | Amyl phosphite                               |
|    | Trimethyl phosphine oxide                    |
|    | Trimethyl phosphine sulfide                  |
|    | Triethyl phosphine oxide                     |
|    | Triethyl phosphine sulfide                   |
| 55 | Tripropyl phosphine oxide                    |
|    | Tripropyl phosphine sulfide                  |
|    | Tributyl phosphite                           |
|    | Lecithin                                     |
|    | Diethyl isoamyl thiophosphinate              |
|    | Diamyl methyl phosphinate                    |
| 60 | Diethyl propyl phosphinate                   |
|    | Amyl diamylphosphinate                       |
|    | Butibutyl alpha hydroxy isopropylphosphinate |
|    | Tri (sulfurized oleyl alcohol) phosphite     |
| 65 | Tri (sulfurized oleyl alcohol) phosphate     |
|    | Trilauryl phosphite                          |
|    | Trilauryl phosphate                          |
|    | Trilauryl thiophosphite                      |
|    | Trilauryl thiophosphate                      |
|    | Trioctadecyl phosphite                       |
| 70 | Trioctadecyl phosphate                       |
|    | Trichlorolauryl phosphite                    |
|    | Trichlorolauryl phosphate                    |
|    | Calcium lauryl phosphite                     |
|    | Aluminum lauryl phosphite                    |
| 75 | Zinc lauryl phosphate                        |

## II. Aromatic

Triphenyl phosphine oxide  
 Triphenyl phosphine sulfide  
 Tritolyl phosphine oxide  
 Tritolyl phosphine sulfide  
 Trixylyl phosphine oxide  
 Trixylyl phosphine sulfide  
 Naphthyl phosphine oxide  
 Naphthyl phosphine sulfide  
 Trifurfuryl thiophosphite  
 Trifurfuryl thiophosphate  
 Monoethyl ditolyl phosphine oxide  
 Monoethyl ditolyl phosphine sulfide  
 Trifuryl phosphine oxide  
 Trifuryl phosphine sulfide  
 Chlorotritolyl phosphine oxide  
 Chlorotritolyl phosphine sulfide  
 Phosphenyl oxide  
 Phosphine-benzene  
 Triphenyl phosphine  
 Triphenyl phosphite  
 Tritertiary amyl phenyl phosphite  
 Tricresyl phosphite  
 Tribeta naphthyl phosphite  
 Tritertiary butyl phosphite  
 Phenyl 1,4 phosphoxane  
 Diethyl phenylphosphinite  
 Diethyl phenyl thiophosphinite  
 Isopropyl diphenylthiophosphinite  
 Phenyl diphenylphosphinite  
 Diethyl paratolylphosphinate  
 Triphenyl phosphine sulfide  
 Triphenyl phosphine oxide  
 P-carboxy phenyl phosphine oxide  
 Propyl benzene dichlor phosphine  
 Butyl benzene dichlor phosphine  
 B-amyl phenoxyethyl phosphite  
 Triamyl phenyl phosphite  
 Trichloro cresyl phosphite  
 Tricresyl phosphate  
 Tricresyl thiophosphite  
 Sodium dicresyl phosphite  
 Sodium dicresyl phosphate  
 Aluminum phenyl thiophosphite  
 Aluminum phenyl thiophosphate

## III. Carbocyclic

Tricyclohexyl phosphite  
 Tricyclohexyl phosphate  
 Trichlorocyclohexyl phosphite  
 Trichlorocyclohexyl phosphate  
 Tricyclohexyl phosphine oxide  
 Tricyclohexyl phosphine sulfide  
 Tetrahydronaphthyl phosphine oxide  
 Tetrahydronaphthyl phosphine sulfide  
 Cyclo-tetramethylene methyl phosphine  
 Cyclo-pentamethylene phosphine

## IV. Reaction products

1. Phosphorized rapeseed oil, formed by reacting rapeseed oil with a reactant selected from the group consisting of phosphorus chlorides, phosphorus oxyhalides, phosphorus oxides, phosphorus sulfides, sodium phosphide and tin phosphide.
  2. Phosphorized castor oil, formed by reacting castor oil with a reactant selected from the group consisting of phosphorus chlorides, phosphorus oxyhalides, phosphorus oxides, phosphorus sulfides, sodium phosphide, and tin phosphide.
  3. Phosphorized hydrocarbon oil made by reacting hydrocarbon oil with  $\text{PSCl}_3$ .
- 10
4. Reaction product of 3 parts of potassium ethyl xanthate and 1 part of phosphorus trichloride.
  5. Reaction product of potassium ethyl xanthate and phosphorus oxychloride.
  6. Reaction product of phenol and phosphorus trichloride.
  7. Reaction product formed by reacting dibutyl tartrate with phosphorus trichloride.
  8. Reaction product formed by reacting phosphorus trichloride with trimethyl citrate.
  9. Reaction product of phosphorus trichloride with paraffin wax.
  10. Reaction product of phosphorus pentoxide with cetyl alcohol.
  11. Reaction product of phosphorus trisulfide with octadecanol.
- Lubricants having added thereto small but effective proportions of both a sulfurized olefin and an organic phosphorus compound possess unexpectedly superior properties. Highly refined lubricants such as solvent-treated Mid-Continent oils having a viscosity index above 93 and Pennsylvania paraffinic oils normally quite 20 corrosive to sensitive bearing metals after a short period of use are rendered stable and non-corrosive by the remarkable antioxidant and inhibiting effect of the combination of addition agents. Furthermore these same oils which are 25 notoriously quick to form lacquers and varnishes on the highly heated metal surfaces contacted by them are rendered practically neutral in respect to formations of lacquer and varnish deposits. The most astonishing feature of this 30 invention, however, is the extent to which the oil inhibited by the combination of inhibitors resists the formation of sludge and sludge-like materials commonly called naphtha and chloroform insolubles even though the oil is used or 35 tested under the most severe and accelerated oxidation conditions. This particular attribute is clearly shown in the modified Underwood tests hereinbelow discussed and in engine tests conducted on oils within the scope of this invention. Furthermore the lubricants of our invention 40 maintain the insoluble constituents and contaminants normally present in a lubricating oil after usage colloidally suspended or in a state other than that deposited on the engine 45 parts in hard, gummy, or varnish-like deposits. For these reasons, the lubricants improved in accordance with this invention are of extraordinary value for the lubrication of the parts within the crankcases of internal combustion engines.
- 50 The foregoing facts were determined by various test procedures which have been devised and are available by which a comparative evaluation of oils with respect to deterioration thereof in service may be obtained in a relatively short 55 period of time. The evidence of the broad utility of inhibitors according to the invention in its intended field of service is afforded by the results of a test method wherein internal combustion engine lubricants comprise the oil environment in which the inhibitors function. This test is one devised in recent years to demonstrate the tendency of motor oils to deteriorate per se and their tendency to corrode bearing surfaces in internal combustion engines 60 wherein the bearings are formed of or surfaced with easily corroded alloys. It is observed that motor oils derived from selected crudes predominantly paraffinic in origin, as well 65 as other oils from other crudes which have been 70 improved by treatment with selective solvents,
- 75

## 11

exhibit a marked tendency toward corrosion of the bearings in question, although in other respects the lubricants are of superior quality. The test, which is known as the "modified Underwood oxidation test," is conducted substantially as follows:

Standard half-bearings of copper-lead and cadmium-silver are supported in a chamber through which air may be circulated. A sheet of lead is placed in the heater chamber. This acts as a catalyst to promote and increase the rate of oxidation and deterioration of the oil. The surfaces of the bearings are exposed for various periods of time to a stream of oil sprayed under pressure continuously upon the corrodible areas. The oil is maintained at a temperature of 350° F. The oil is recirculated over the bearing surfaces to simulate surface conditions in an automotive crankcase. The oil deterioration is ascertained by determining the neutralization number of the oil after a test run as well as other physical and chemical changes such as the increase of viscosity, the carbon residue, and the resin and sludge content. The measure of corrosion is taken as the loss in weight of the bearings per unit of exposed corrodible surface.

The foregoing test, which has been determined to be very well correlated with actual crankcase service conditions, was made upon unblended oils, blends of oil with sulfurized olefins, blends of oil with organic phosphorus compounds, and blends of oil with combinations of sulfurized olefin and various organic phosphorus compounds.

The results of these tests clearly revealed the properties and advantages of lubricants prepared according to this invention, particularly if the lubricant is to be used in the crankcase of an internal combustion engine.

## THE MODIFIED UNDERWOOD TESTS

An unblended 400 pale oil solvent treated to a viscosity index of 98 by treating with 3 parts furfural to 1 part oil at 250° F. and having a Saybolt universal viscosity of 61.0 seconds at 210° F. was tested in the modified Underwood oxidation apparatus. The following determinations were made:

## Test 1.—Blank oil, unblended 400 pale

| Hours.....                                           | 2    | 3     | 4     | 5     |
|------------------------------------------------------|------|-------|-------|-------|
| Corrosion Cu-Pb Gms.....                             | 0.03 | 0.24  | 0.36  | 0.50  |
| Corrosion Cd-Ag Gms.....                             | 0.27 | 1.03  | 1.64  | 2.43  |
| Neutralization No.....                               | 3.1  | 5.1   | 6.0   | 7.0   |
| Petroleum Naphtha Insoluble, per cent by weight..... | 0.06 | 0.08  | 0.08  | 0.09  |
| Chloroform Insoluble, per cent.....                  | 0.06 | 0.07  | 0.07  | 0.07  |
| Viscosity Sec. Saybolt, 210° F. (61.0).....          | 74.0 | 89.6  | 111.4 | 149.6 |
| Ramsbottom Carbon Residue, per cent.....             | 0.5  | 1.02  | 1.56  | 2.55  |
| Resin, per cent.....                                 | 8.9  | 14.92 | 20.94 | 27.26 |

It is apparent that this oil failed rapidly, corrosion being under way at 2 hours with a heavy Cd-Ag loss after 5 hours and a viscosity increase of 88.6 S. S. U. seconds after 5 hours.

A sample of the same oil was blended with 0.015 per cent sulfur in the form of sulfurized olefin, the olefin having been derived from petroleum wax. The following determinations were made:

12  
Test 2.—Oil plus 0.015% sulfur in the form of sulfurized olefin

| Hours.....                                           | 12    | 14    | 16    | 18    |
|------------------------------------------------------|-------|-------|-------|-------|
| Corrosion Cu-Pb Gms.....                             | 0.00  | 0.56  | 1.17  | 1.55  |
| Corrosion Cd-Ag Gms.....                             | 1.27  | 2.05  | 2.93  | 4.54  |
| Neutralization No.....                               | 8.1   | 10.5  | 10.8  | 10.5  |
| Petroleum Naphtha Insoluble, per cent by weight..... | 0.10  | 0.14  | 0.08  | 0.08  |
| Chloroform Insoluble, per cent.....                  | 0.08  | 0.12  | 0.06  | 0.06  |
| Viscosity, Seconds Saybolt, 210° F. (61.0).....      | 86.3  | 102.8 | 119.4 | 136.3 |
| Carbon Residue, per cent.....                        | 2.2   | 3.3   | 4.6   | 6.0   |
| Resin, per cent.....                                 | 19.72 | 21.74 | 27.36 | 30.87 |

15 The test reveals that this oil was much better than the unblended oil, no copper-lead corrosion having occurred until after nearly 14 hours; however the cadmium-silver half-bearing was badly corroded in 12 hours, and the acid content of the oil was high. The viscosity of the oil had been increased by use to such an extent that after 18 hours it was 75.1 seconds Saybolt more viscous at 210° F. than was the original oil. The resin content of the oil was also high.

20 25 A sample of the same oil as was tested in Test 1 and used as the base oil in Test 2 was blended with 0.5 per cent triphenyl phosphite. The following determinations were made:

## 30 Test 3.—Oil plus 0.5% triphenyl phosphite

| Hours.....                                           | 10½  | 13½  | 16½   | 19½   |
|------------------------------------------------------|------|------|-------|-------|
| Corrosion Cu-Pb Gms.....                             | 0.00 | 0.00 | 0.14  | 0.42  |
| Corrosion Cd-Ag Gms.....                             | 0.00 | 0.00 | 1.01  | 2.36  |
| Neutralization No.....                               | 0.5  | 0.8  | 5.0   | 6.0   |
| Petroleum Naphtha Insoluble, per cent by weight..... | 0.02 | 0.03 | 0.03  | 0.03  |
| Chloroform Insoluble, per cent.....                  | 0.02 | 0.03 | 0.03  | 0.03  |
| Viscosity, Seconds Saybolt 210° F. (61.0).....       | 61.8 | 62.6 | 87.7  | 132.4 |
| Carbon Residue, per cent.....                        | 0.14 | 0.23 | 1.21  | 2.69  |
| Resin, per cent.....                                 | 2.99 | 3.85 | 21.35 | 32.48 |

45 The test indicates that this oil is greatly improved as compared to the unblended oil in that no corrosion had occurred at 13½ hours; however at 16½ hours the oil had seriously deteriorated to the point where it was very corrosive to cadmium-silver alloys and quite corrosive to copper-lead alloys, the acid content of the oil having risen to an alarming ratio; and the resin content was very high.

50 55 A sample of oil, the same as used in Test 1 and as base stock for the oils tested in Tests 2 and 3, was blended with 0.015 per cent sulfur in the form of sulfurized olefin in which the olefin was obtained by halogenating and dehydrohalogenating paraffin wax and 0.5 per cent triphenyl phosphite. The following determinations were made.

## 65 Test 4.—Oil plus 0.015 per cent sulfur and 0.5 per cent triphenyl phosphite

| Hours.....                                           | 10   | 15   | 20   | 25   |
|------------------------------------------------------|------|------|------|------|
| Corrosion Cu-Pb Gms.....                             | 0.00 | 0.00 | 0.01 | 0.08 |
| Corrosion Cd-Ag Gms.....                             | 0.00 | 0.00 | 0.02 | 0.04 |
| Neutralization No.....                               | 0.4  | 0.6  | 1.2  | 2.2  |
| Petroleum Naphtha Insoluble, per cent by Weight..... | 0.04 | 0.03 | 0.05 | 0.16 |
| Chloroform Insoluble, per cent.....                  | 0.03 | 0.03 | 0.04 | 0.14 |
| Viscosity, Seconds Saybolt 210° F. (61.0).....       | 61.4 | 63.0 | 64.4 | 66.8 |
| Carbon Residue, per cent.....                        | 0.19 | 0.27 | 0.45 | 0.76 |
| Resin, per cent.....                                 | 3.18 | 3.89 | 5.48 | 7.42 |

The examination of this oil proved it to be practically noncorrosive at 25 hours, only 0.08 gram of the copper-lead half-bearing having been lost and only 0.04 gram of the cadmium-silver half-bearing having been lost. The acid content of the oil was relatively low. The carbon residue and resin content were very low. The viscosity of the oil was practically unaffected.

A study of the above results graphically reveals that we have accomplished the objects of our invention. We have produced a lubricant which may be used for unusually long periods of time under severe operating conditions in the crank-case of an internal combustion engine without danger of bearing loss through corrosion. We have made available a lubricant which is not readily oxidized to form sludges and lacquer formations. The lubricant prepared in accordance with our invention does not become viscous with use under severe conditions as does the lubricant which has not been blended with the additives which are within the ambit of this invention. The results obtained by the combination of the two classes of additives are unexpectedly greater and more beneficial than would be expected from the study of the effect of each of the additives added separately to oil. We have no adequate theory to explain this enhanced oil but believe the phosphorus compounds act as antioxidants to prevent the early oxidation and decomposition of the oil but that their effect is lost after a short time of severe operating use and also impart that characteristic above referred to as detergency to an oil while the sulfur compound is not a true antioxidant but only as anticorrosive properties by (a) reacting with the corrosive products of oxidation, corrosion, and decomposition to render them inert and (b) reacting with the catalytically active material such as metallic oxides and salts rendering them inert catalytically. We believe the combined effect of the addition of small amounts of sulfurized olefins, prepared by halogenating and dehalogenating narrow-cut petroleum fractions, and a small amount of an organic phosphorus compound is to produce an oil stabilized against oxidation and deterioration for a longer period of time and further beneficially affected after it has started to oxidize and decompose by being maintained in a noncorrosive and catalytically inert condition thereby producing an oil capable of use for prolonged periods of time under severe conditions without serious change in lubricating ability or damage to the readily corroded bearing metals. We do not intend to be bound by our theory but prefer to base our invention upon the improved effect which may be demonstrated.

Even though the joint action of the sulfur compound and phosphorus compound gives results unexpected from a combination of the actions of the two compounds separately, we have found that the ratio of phosphorus to sulfur in the finished lubricant should be fairly well controlled for most satisfactory results. Generally speaking, we prefer to use combinations of sulfurized compounds and organic phosphorus compounds in which at least 10 per cent but not more than 70 per cent of the combined weight of the additives is an organic phosphorus compound. This particular range, however, is not critical; and smaller or larger proportions may be used and, in some cases, may be found more desirable.

In addition to the above-mentioned improvements, the lubricants prepared according to this invention, especially those containing a relatively

higher percentage ratio of the additives, have a high film strength.

The lubricants containing a substantial proportion of some of the organic phosphorus compounds exhibit increased detergency and peptizing character and are of particular value for use in Diesel engine crankcases where the presence of soot and products of combustion constitutes a serious problem.

10 The lubricating oil portion of the blends of our invention may be so-called mineral or hydrocarbon oils which may be poorly, moderately, or highly refined, paraffinic or naphthenic, or may consist wholly of or contain only in part certain fatty oils, including corn oil, soy bean oil, lard oil, and like oils of lubricating viscosity. The blends may contain volatilized oils or synthetic oils of lubricating viscosity. Soap-thickened or otherwise thickened oils used as greases may be employed. Addends for other purposes such as a pour point depressant may be present.

Since the phosphorus compounds have varying degrees of solubility in various hydrocarbon oils in some cases, it may be necessary to use a mutual solvent for the compound and the oil in order to properly incorporate the phosphorus compound into the oil.

Finally and again it may be said that very small amounts of these compounds are very effective when added to a lubricating oil. A wide range may be employed. As little as 0.001 per cent of the combination of these compounds appreciably improves the oil. As much as 20 per cent of the combination of these compounds may be used in gear lubricants and the like.

It will be understood that certain features and subcombinations are of utility and may be employed without reference to other features and subcombinations. This is contemplated by and 30 is within the scope of our claims. It is further obvious that various changes may be made in details within the scope of our claims without departing from the spirit of our invention. It is 40 therefore to be understood that our invention is 45 not to be limited to the specific details shown and described.

Having thus described our invention, we claim:

1. A lubricant comprising in combination a major proportion of an oil of lubricating viscosity and a minor proportion, sufficient to improve the properties of the oil as regards corrosion and oxidation of sulfurized monomeric olefin, said olefin being obtained from a narrow-cut petroleum fraction and a minor proportion of an organic phosphorus compound.

2. A lubricant comprising in combination a major proportion of oil of lubricating viscosity and a minor proportion, sufficient to improve the properties of the oil as regards corrosion and oxidation of sulfurized olefin, said olefin being formed by halogenating and dehydrohalogenating petroleum wax, and an organic phosphorus compound.

3. A lubricant comprising in combination a major proportion of oil of lubricating viscosity and a minor amount, sufficient to improve the properties of the oil as regards corrosion and oxidation of sulfurized olefin, said olefin being formed by halogenating a petroleum wax, separating the monochlor wax from the unchlorinated wax and the more highly chlorinated wax, and dehydrohalogenating the relatively pure monochlor wax, and a minor proportion of an organic phosphorus compound.

4. A lubricant comprising in combination a major proportion of oil of lubricating viscosity and a minor proportion, sufficient to improve the properties of the oil as regards corrosion and oxidation of a sulfurized olefin, said olefin being formed by chlorinating a petroleum wax, separating the monochlor wax from the more highly chlorinated wax and the unchlorinated wax, and dehydrohalogenating the relatively pure monochlor wax, and a minor proportion of organic phosphorus compound.

5. A lubricant comprising in combination a major proportion of oil of lubricating viscosity and a minor proportion, sufficient to improve the properties of the oil as regards corrosion and oxidation of a sulfurized olefin, said olefin being obtained by chlorinating a relatively pure petroleum wax to the monochlor compound, separating the monochlor wax from the crude-chlorination mixture and dehydrohalogenating, the sulfurizing being by means of an agent selected from the group consisting of elemental sulfur, chlorides of sulfur, sulfides of phosphorus, and a minor proportion of an organic phosphorus compound.

6. A lubricant comprising in combination a major proportion of oil of lubricating viscosity and a minor proportion, sufficient to improve the properties of the oil as regards corrosion and oxidation of sulfurized olefin, said olefin being formed by chlorinating a petroleum paraffin wax to the monochlor compound, separating the monochlor compound from the crude-chlorination mixture and dechlorinating by heating in the presence of a catalyst, the sulfurizing being by means of elemental sulfur, and a minor proportion of an organic phosphorus compound.

7. A lubricant comprising in combination a major proportion of oil of lubricating viscosity and a minor proportion, sufficient to improve the properties of the oil as regards corrosion and oxidation of sulfurized olefin, said olefin being formed by chlorinating a petroleum wax to the monochlor wax, separating the monochlor wax from the crude-chlorination mixture, dechlorinating, the sulfurization being by means of a sulfur compound selected from the group consisting of sulfides of phosphorus and chlorides of sulfur, and a minor proportion of an organic phosphorus compound.

8. A lubricant comprising in combination a major proportion of oil of lubricating viscosity, a minor proportion, sufficient to improve the properties of the oil as regards corrosion and oxidation of sulfurized olefin, said olefin being obtained by chlorinating a paraffin wax, and dechlorinating, and a minor proportion of an aliphatic phosphorus compound.

9. A lubricant comprising in combination a major proportion of oil of lubricating viscosity and a minor proportion, sufficient to improve the properties of the oil as regards corrosion and oxidation of sulfurized olefin, said olefin being obtained from paraffin wax by halogenation and dehalogenation, and a minor proportion of an aromatic phosphorus compound.

10. A lubricant comprising in combination a major proportion of lubricating oil and a minor proportion, sufficient to improve the properties of the oil as regards corrosion and oxidation of sulfurized olefin, said olefin being obtained by halogenating a paraffin wax and dehalogenating, and a minor proportion of heterocyclic phosphorus compound.

11. A lubricant comprising in combination a major proportion of oil of lubricating viscosity and a minor proportion, sufficient to improve the properties of the oil as regards corrosion and oxidation of sulfurized olefin, said olefin being obtained from petroleum wax by halogenation and dehalogenation, and a minor proportion of phosphorized mineral oil.

12. A lubricant comprising in combination a major proportion of oil of lubricating viscosity and a minor proportion, sufficient to improve the properties of the oil as regards corrosion and oxidation of sulfurized olefin, said olefin being obtained from petroleum wax by halogenation and dehalogenation, and a minor proportion of ester of phosphorus acid.

13. A lubricant comprising in combination a major proportion of oil of lubricating viscosity and a minor proportion, sufficient to improve the properties of the oil as regards corrosion and oxidation of sulfurized olefin, said olefin being obtained by halogenating and dehalogenating paraffin wax, and a minor proportion of a phosphine.

14. A lubricant comprising in combination a major proportion of oil of lubricating viscosity and a minor proportion, sufficient to improve the properties of the oil as regards corrosion and oxidation of sulfurized olefin, said olefin being obtained by halogenating and dehalogenating paraffin wax, and a minor proportion of an organic phosphate.

15. A lubricant comprising in combination a major proportion of oil of lubricating viscosity and a minor proportion, sufficient to improve the properties of the oil as regards corrosion and oxidation of sulfurized olefin, said olefin being obtained by halogenating and dehalogenating paraffin wax, and a minor proportion of an organic phosphite.

16. A lubricant comprising in combination a major proportion of oil of lubricating viscosity and a minor proportion, sufficient to improve the properties of the oil as regards corrosion and oxidation of sulfurized olefin, said olefin being obtained by halogenating and dehalogenating paraffin wax, and a minor proportion of triphenyl phosphite.

17. A lubricant comprising in combination a major proportion of oil of lubricating viscosity and a minor proportion, sufficient to improve the properties of the oil as regards corrosion and oxidation of sulfurized olefin, said olefin being obtained by halogenating and dehalogenating paraffin wax, and a minor proportion of triethyl phosphine oxide.

18. A lubricant comprising in combination a major proportion of oil of lubricating viscosity and a minor proportion, sufficient to improve the properties of the oil as regards corrosion and oxidation of sulfurized olefin, said olefin being obtained by halogenating and dehalogenating paraffin wax, and a minor proportion of lecithin.

19. A lubricant comprising in combination a major proportion of oil of lubricating viscosity and a minor proportion, sufficient to improve the properties of the oil as regards corrosion and oxidation of sulfurized relatively high molecular weight olefin and a minor proportion of an organic phosphorus compound.

20. A lubricant comprising in combination a major proportion of oil of lubricating viscosity and a minor proportion, sufficient to improve the properties of the oil as regards corrosion and oxidation of sulfurized monomeric olefin, said olefin

17

being obtained from petroleum, and a minor proportion of an organic phosphorus compound.

BERT H. LINCOLN.

GORDON D. BYRKIT.

WALDO L. STEINER.

## REFERENCES CITED

The following references are of record in the file of this patent:

## UNITED STATES PATENTS

|           |         |              |
|-----------|---------|--------------|
| Number    | Name    | Date         |
| 2,167,867 | Benning | Aug. 1, 1939 |

18

| Number       | Name           | Date           |
|--------------|----------------|----------------|
| 2,218,132    | Lincoln et al. | Oct. 15, 1940  |
| 2,226,543    | Ashburn        | Dec. 31, 1940  |
| 2,231,301    | Smith          | Feb. 11, 1941  |
| 5 2,242,260  | Prutton        | May 20, 1941   |
| 2,260,303    | Engelke        | Oct. 28, 1941  |
| 2,278,719    | Davis et al.   | Apr. 7, 1942   |
| 2,285,854    | Downing et al. | June 9, 1942   |
| 2,296,037    | Kaufman        | Sept. 15, 1942 |
| 10 2,313,248 | Lincoln et al. | Mar. 9, 1943   |
| 2,348,080    | Lincoln et al. | May 2, 1944    |
| 2,353,837    | Loane          | July 18, 1944  |